

# UNITED STATES PATENT OFFICE.

MARC CHIRADE AND JOSEPH CANAC, OF PARIS, FRANCE.

## PROCESS FOR DIRECT NICKELING OF ALUMINUM OR ALLOYS CONTAINING ALUMINUM.

1,030,972.

Specification of Letters Patent.

Patented July 2, 1912.

No Drawing.

Application filed November 6, 1911. Serial No. 658,734.

*To all whom it may concern:*

Be it known that we, MARC CHIRADE and JOSEPH CANAC, engineers, citizens of the French Republic, residing in Paris, France, with post-office address care of J. P. Bonnicart, 16 Place de la République, Paris, France, have invented a new and useful Process for Direct Nickelizing of Aluminium or Alloys Containing Aluminium, of which the following is a specification.

The invention relates to improvements in processes of direct aluminium nickelizing.

The object of the invention is to enable any article of pure aluminium or alloy containing same, to be nickelized directly. This object is attained by the following process: 1°. Immerse the article to be nickelized in tepid water, next wash it in ordinary water containing 2 per cent of cyanid of potassium.

20 The article is left about 30 seconds in the latter composition and then washed with very clean water. 2°. Immerse the article, after the above treatment, in the following composition: hydrochloric acid  $\frac{1}{2}$  liter, dis-

tilled water  $\frac{1}{2}$  liter, chlorid of iron, 1 gram. 25 3°. Wash the article in clean water and immerse in nickel bath by furnishing an electrical current of three volts; after five minutes, again wash in boiling water, preferably, and finally dry by any convenient 30 means.

We claim:

The process for direct nickelizing of aluminium articles or alloy containing aluminium, consisting in subjecting the aluminium or 35 alloy to a washing bath composed of water and cyanid of potassium, next immersing the article in a scouring bath formed of hydrochloric acid, distilled water and chlorid of iron and finally placing it in a nickel bath 40 under electrical current of three volts, all substantially as set forth.

MARC CHIRADE.  
JOSEPH CANAC.

Witnesses:

JEAN PAUL BONNICART,  
DEAN B. MASON.